

## UNITED STATES PATENT OFFICE

1,963,829

## PRODUCING HIGH VACUA

Hugh S. Cooper, Cleveland, Ohio, assignor to  
Kemet Laboratories Company, Inc., a corpora-  
tion of New York

No Drawing. Application December 5, 1931,  
Serial No. 579,855

11 Claims. (Cl. 250—27.5)

High vacua are customarily produced in thermionic tubes and the like by removing the greater part of the gas from the device by mechanical pumping, and cleaning up the residual traces of gas by the use of a clean-up agent or "getter" which, it is believed, fixes the residual gases by both chemical and physical action. My invention relates to this process of producing high vacua, and although it is primarily directed to the production of vacua in thermionic valves and similar devices, it is applicable to the production of vacua generally.

Clean-up agents are customarily placed within the device to be evacuated and later volatilized by inductive electric heating; the volatilizing step being commonly termed "flashing". The time and temperature required to flash the clean-up agent are frequently very important factors in the manufacture of thermionic devices, especially when the manufacturing steps, which include flashing, are performed by automatic machinery, which is usually the case.

The objects of my invention are to provide a series of new clean-up agents characterized by the ease and rapidity with which they may be flashed, and to provide a method by which the time required to flash known clean-up agents may be reduced. I obtain these and other objects by taking advantage of the intense exothermic reaction that results when aluminum alloys with nickel and cobalt.

According to my invention a clean-up agent is prepared by placing in mutual contact one of the following combinations: a metal predominantly of nickel, a metal predominantly of aluminum, and a clean-up material; or a metal predominantly of nickel, and an aluminum alloy of a clean-up material; or a metal predominantly of aluminum, and a nickel alloy of a clean-up material. Pure nickel and aluminum are generally preferable.

It is to be understood herein that cobalt is the substantial equivalent of nickel wherever the latter is used.

The clean-up material used in the clean-up agent may be any metal or alloy thereof which is effective when volatilized within an envelope to fix residual traces of gas therein. For example, the alkaline earth metals and their alloys such as barium, strontium, calcium, barium-silicon alloy, and the like are suitable as a clean-up material.

According to one application of my invention, clean-up agents are prepared by closely associating metallic nickel with an aluminum alloy, either

ductile or friable, containing a clean-up material such as an alkaline earth metal. One method of application is to flash while in mutual contact a piece of metal comprising chiefly nickel and another piece of metal comprising the aluminum alloy or a plurality of laminae built up from alternate pieces of the two metals. The aluminum alloy may be in the form of ductile metal or a powdered friable alloy, and the latter may conveniently be compressed to a solid tablet. Another method of application, best suited to the friable aluminum alloys, is to flash an intimate mixture of powdered aluminum alloy and powdered nickel. This mixture may also be compacted into a tablet or the like if it is so desired.

Another application of my invention consists in closely associating nickel and aluminum with a clean-up material such as an alkaline-earth metal or an alloy thereof, for example an alloy of barium and silicon. The nickel, aluminum and clean-up material may be powdered and intimately mixed, or closely associated in any similar suitable manner.

A further application of my invention consists in associating aluminum with an alloy of nickel containing a clean-up material, for instance an alloy of nickel and barium. The aluminum and the alloy may both be solid ductile pieces, or both powdered, or either one powdered and the other a solid ductile piece.

The advantages of my invention are demonstrated by experiments which I have made. For example, I prepared a friable alloy comprising aluminum and barium in approximately equal proportions. A clean-up agent was prepared from this material, and introduced into a glass envelope, the envelope was mechanically-evacuated and the agent flashed. About 12 seconds flashing time was required. A portion of the same barium-aluminum alloy was then mixed in powdered form with about an equal weight of powdered nickel, a clean-up agent compressed and compacted therefrom, and the agent flashed under conditions substantially identical with those previously used. Only about 8 seconds flashing time was required for the alloy-nickel agent. The barium given off by the latter agent apparently is exceedingly pure, and the mirror formed by the agent upon the wall of the bulb was brighter and more silvery than is ordinarily secured when barium-containing agents are used. The barium-aluminum alloy per se is not a part of this invention.

In another experiment I prepared a barium-silicon alloy containing about equal proportions

of barium and silicon. A getter prepared from this alloy was flashed in about 12 seconds. A getter prepared by pulverizing some of this same alloy and adding pulverized nickel and aluminum, 5 in the following approximate proportions: nickel 50%, barium-silicon alloy 45%, aluminum 5%, was easily flashed under the same conditions in slightly more than 8 seconds.

Similarly, the time required to flash an alloy 10 of nickel and barium may be decreased by closely associating aluminum with the alloy.

When alkaline earth metal alloys of aluminum or nickel are used, it is desirable to have at least 5% of the alkaline earth metal present in the 15 alloy, so as to avoid the necessity of using an excessive amount of alloy to secure satisfactory clean-up of gases.

Although I have described my invention with specific reference to the alkaline earth metals, 20 as the clean-up materials, other clean-up materials may be used as substantial equivalents for the purpose. It is evident that the clean-up material may comprise any number of suitable metals in any proportions, and that they may be alloyed with either the nickel or the aluminum, 25 or be unalloyed with either. The nickel and the aluminum must not be alloyed with each other, that is to say, they must be physically separable.

30 I claim:

1. A clean-up agent suited for use in producing vacua which comprises nickel, aluminum and a clean-up material, the nickel being alloyed with the clean-up material and the aluminum being physically separable from the said alloy.
2. A clean-up agent suited for use in producing high vacua which comprises two metals in mutual contact, one metal being predominantly of aluminum and the other being an alloy of nickel with at least one clean-up material such as barium, strontium or calcium.
3. A clean-up agent suited for use in producing high vacua which comprises two metals in mutual contact, one of said metals being substantially pure aluminum and the other being an alloy of nickel with at least one of the metals barium, strontium, calcium.
4. A clean-up agent suited for use in producing high vacua which comprises aluminum and 50 an alloy of nickel with at least 5% of barium;

55

60

65

70

75

the nickel and aluminum alloy being in mutual contact.

5. A clean-up agent suited for use in producing high vacua which comprises an intimate mixture of subdivided nickel, subdivided aluminum, and subdivided alloy of barium and silicon. 80

6. A clean-up agent suited for use in producing high vacua which comprises an intimate mixture of powdered nickel and a powdered friable alloy of aluminum with at least one of 85 the alkaline earth metals barium, strontium, calcium.

7. A clean-up agent comprising an intimate mixture of powdered nickel and a powdered friable alloy comprising approximately equal 90 parts of aluminum and barium.

8. Process of producing a high vacuum which comprises introducing into an envelope a clean-up agent consisting of nickel, aluminum and a clean-up material, the nickel and aluminum being physically separable; mechanically evacuating 95 said envelope; and alloying the nickel with the aluminum, thereby volatilizing at least part of the clean-up material in said agent.

9. Process of producing a high vacuum which 100 comprises introducing into an envelope a clean-up agent consisting of a metal predominantly of aluminum in contact with an alloy of nickel containing clean-up material; mechanically evacuating said envelope; and alloying the nickel 105 with the aluminum, thereby volatilizing at least part of the clean-up material in said agent.

10. Process of producing a high vacuum which comprises introducing into an envelope a clean-up agent consisting of two metals in mutual 110 contact, one being composed predominantly of nickel and the other being an alloy of aluminum with at least one of the group: barium, strontium and calcium; mechanically evacuating said envelope; and alloying the nickel with the aluminum, thereby volatilizing at least part of the 115 clean-up material in said agent.

11. A clean-up agent suited for use in producing vacua which comprises a plurality of laminae, alternate laminae consisting of a metal 120 predominantly aluminum, and the remaining laminae consisting of an alloy comprising nickel and a clean-up material.

HUGH S. COOPER. 125

130

135

140

145

150